

1

3,443,946

## PHOTOGRAPHIC MATERIAL HAVING A ROUGHENED PROTECTIVE LAYER

Herbert Grabhöfer, Cologne-Flittard, and Günter Meinhart, Leverkusen, Germany, assignors to Agfa Aktiengesellschaft, Leverkusen, Germany, a corporation of Germany

No Drawing. Filed May 13, 1965, Ser. No. 455,605  
Claims priority, application Germany, June 4, 1964,

A 46,219

Int. Cl. G03c 1/72

U.S. Cl. 96—50

4 Claims

### ABSTRACT OF THE DISCLOSURE

Protective layer for photographic material, which layer has a water-permeable binder containing particles of an acrylonitrile polymer plasticized with a beta-cyanoethyl ether of a polyhydric aliphatic alcohol or a phosphoric acid ester of pentaerythritol.

The invention relates to a photographic material having a transparent roughened protective layer.

It is known to provide photographic layers with protective coatings for protection against scratching and other harmful influences. Materials of very different chemical constitutions are used for these coatings. Generally, the light-sensitive emulsion side is coated with an outer thin gelatine layer. Other water-soluble or alkali-soluble film formers, which are used in a known manner for this purpose, are for example other proteins, such as casein, partially hydrolyzed polyvinyl acetate, polyvinyl alcohol, polyvinyl phthalate, cellulose acetate phthalate and substances of high molecular weight which are of similar structure. All these substances have the disadvantage that, when they dry, they produce more or less smooth surfaces which are undesirable for many uses in the photographic art. For example, photographic materials provided with such protective coatings can only be retouched and written on with difficulty. Furthermore, Newton's rings are formed on printing or on projection. Smooth surfaces also have a tendency to become electrostatically charged, causing local blackening on the light-sensitive layer. Many experiments have been carried out in an attempt to eliminate these disadvantage properties of smooth protective layers. Thus, it is known to incorporate starch in finely divided form into light-sensitive photographic layers. In addition, water-insoluble plastic particles of polystyrene, polyesters and similar synthetic materials of high molecular weight have been used for roughening the surface. It is true that all these measures lead to a detectable improvement in the writing capacity and reduce the formation of Newton's rings and electrostatic charges, but they also introduce other disadvantages, for example, a general clouding of the layers, which frequently shows in the form of spots, sedimentation of the plastic dispersion during casting and finally matting effects, which are particularly undesirable when producing transparent pictures.

It is an object of the invention to provide a protective layer which does not have the aforesaid disadvantages and which, with simple composition and processing, prevents the formation of Newton's rings and electrostatic charging and enables the photographic image to be written on or retouched.

It has now been found that a transparent protective layer with a roughened surface of the composition as indicated below, applied as an outer layer to the front and/or back of a light-sensitive photographic material, has properties which satisfy all requirements.

2

The protective layer according to the invention contains the following components:

#### (I) Film-forming binding agent

Suitable for this purpose are numerous polymers which must be pervious to water and are capable of forming thin films. It is preferred to use gelatin, but this can be wholly or partially replaced by other products, such as casein, albumin, polyvinyl alcohol, partially hydrolyzed polyvinyl acetate, preferably having at the last 10 mol percent vinylacetate units, polyamides, polyvinyl pyrrolidone, carboxymethyl cellulose, alginic acid and derivatives thereof, such as salts, particularly alkali metal salts, esters preferably with lower aliphatic alcohols having up to 5 carbon atoms, or amides, carragenates and similar substances.

#### (II) Polymer containing nitrile groups

This component is heterogeneously distributed in the protective layer, but cannot be detected optically in the final layer by simply looking therethrough, or can only be detected by a very weak opalescence. The polymers contain acrylonitrile or methacrylonitrile units in polymerized form, advantageously in quantities of at least 50 mol percent.

Polyacrylonitrile or polymethacrylonitrile, more especially the former, are preferred. Suitable as components for copolymers are for example acrylic acid esters or methacrylic acid esters with an aliphatic alcohol having up to about 6 carbon atoms, vinyl acetate, alkylvinyl ethers, of which the alkyl group contains up to 4 carbon atoms, and also N-vinylpyrrolidone, N-vinylimidazole, vinyl pyridine, acrylamide or methacrylamide. The grain size of the polymers to be used should be 1 to 25 $\mu$ , advantageously 1 to 5 $\mu$ .

#### (III) Plasticizer

The plasticizer prevents the optical detection of the particles of Component II. This effect is based on the fact that the smaller polymer particles, which would cause a clouding and matting, are completely solvated, but the larger particles are only softened on the surface.

This effect is restricted to plasticizers, which are characterized by a content of  $\beta$ -cyanethoxy-and/or ethylene oxide groups. The following types of plasticizers exhibit particular utility:

(A)  $\beta$ -Cyanoethyl ethers of polyhydric and advantageously dihydric to tetrahydric aliphatic alcohols advantageously containing up to 10 carbon atoms, for example, glycol, glycerine, pentaerythritol, diethylene glycol, triethylene glycol and the like. Suitable products are described in U.S. Patent 2,401,607. The following are mentioned as example:



(5) Di- $\beta$ -cyanoethyl ethers of pentaerythritol, of which the residual 2 hydroxyl groups have been reacted by acetalization with a ketone or aldehyde to form a

cyclic ether grouping of the m-dioxane type. These compounds have the general formula:



wherein  $R_1$  and  $R_2$  represent hydrogen, alkyl advantageously containing up to 6 carbon atoms, aryl, advantageously phenyl, or heterocyclic radicals, such as pyrimidine or morpholine. These groups, more especially the phenyl rings or heterocyclic radicals, can contain further substituents, such as low alkyl or alkoxy having up to 3 carbon atoms or halogen atoms such as chlorine and the like.

Suitable compounds and the preparation thereof are described in British patent specification No. 926,689 and the following is mentioned by way of example:



(B) Phosphoric acid esters of pentaerythritol of the formula



in which formula,  $R_3$  and  $R_4$ , which may be the same or different, represent alkyl, cyanoalkyl and especially cyanoethyl, with up to 18 carbon atoms, or aryl such as phenyl, and  $n=1-20$ , advantageously 1-10. These compounds and the preparation thereof are described in British patent specification No. 922,251, and Belgian patent specification No. 636,304. The following are mentioned as examples:



The protective layers consisting of the above three components advantageously should contain (per 100 parts of the film-forming component I such as gelatine), 5-200 parts of plasticizer and 0.5 to 10 parts of polymer. More especially suitable are those mixtures which contain 10-50 parts of plasticizers and 1-3 parts of polymer II, per 100 parts of gelatine.

In carrying out the process according to the invention, the aqueous dispersions of the polymers are incorporated by stirring, together with the plasticizers, into the binder solution which can be provided with the usual casting additives. Using this casting solution, the photographic film material is coated on the light-sensitive silver halide emulsion layer and/or on the rear side by known casting methods.

The mixing ratio between polymer proportion and plasticizer proportion depends on the required degree of roughness and can be 1:1 to 1:100, advantageously 1:5 to 1:20. The mixture of these substances is added in such a concentration to the outer protective layer that 0.1 to 5 g. per square metre are contained in the dried layer.

The protective layers should have a thickness of about 0.5 to 15 $\mu$ .

The protective layers of the invention have no deleteri-

ous effect on the light-sensitive layers and can be used with all types of black-and-white and color photographic materials, phototechnical materials or photographic elements, which are to be used for making X-ray images.

The protective layers can be applied onto silver halide emulsion layer, filter layers, anti-halo layers, non-curling layers and the like.

There is no dependence on the composition and the number of the layers of the material coated.

10

#### EXAMPLE 1

To 1 litre of 1% aqueous gelatine solution ready for casting, there are added 30 cc. of 10% aqueous solution of plasticizer 1 and 1.5 cc. of a 10% aqueous polyacrylonitrile suspension (prepared by the process described in German Patent 1,058,835) and intensively mixed. This casting solution is applied to that side of a photographic film which contains the light-sensitive gelatine-silver halide emulsion layer and dried. A transparent film is obtained, which layer can be satisfactorily written on, and which has practically no tendency to become electrostatically charged.

30

50 cc. of a 10% aqueous solution of plasticizer 3 and 3 cc. of an aqueous suspension of a copolymer, consisting of 60 mol percent of acrylonitrile units and 40 mol percent of methyl methacrylate emulsion (prepared by the process of German Patent No. 1,058,835) are mixed and added to 1 litre of a 1% aqueous gelatine

35

#### EXAMPLE 2

50 cc. of a 10% aqueous solution of plasticizer 3 and 3 cc. of an aqueous suspension of a copolymer, consisting of 60 mol percent of acrylonitrile units and 40 mol percent of methyl methacrylate emulsion (prepared by the process of German Patent No. 1,058,835) are mixed and added to 1 litre of a 1% aqueous gelatine

55

solution which is ready for casting. This solution is cast onto the silver halide emulsion layer and the rear of a photographic material. The dried layers are free from Newton's rings when in contact with glass.

#### EXAMPLE 3

60 35 cc. of a 10% aqueous solution of plasticizer 7 and 15 cc. of a 10% aqueous solution of plasticizer 9 are mixed with 2 cc. of an aqueous 10% polyacrylonitrile suspension and added to 1 litre of a 1.5% gelatine solution. This mixture is cast on both sides to the silver halide emulsion layers of a photographic X-ray film. This film can be satisfactorily written on and is characterized by an excellent antistatic action, by comparison with a film material having a pure gelatine protective layer.

65 70 After air-conditioning specimens of the film at 35% relative air humidity and 20° C., the electrostatic charging in v./cm. is measured with a rotating field strength measuring instrument according to Schwenkhausen and the electric surface resistivity in ohms is measured with a knife-edge instrument.

## RESULT

|                                 | Charging capacity (v./cm.) | Surface resistivity (10 <sup>12</sup> Ω) |
|---------------------------------|----------------------------|------------------------------------------|
| Control specimen                | +420                       | 13                                       |
| Specimen according to Example 3 | +5                         | 1.5                                      |

5

We claim:

1. In a photographic material having a protective outer layer of a water-permeable binder containing particles of an acrylonitrile polymer having at least 50 mol percent acrylonitrile or methacrylonitrile and a grain size 1 to 25, the improvement according to which the particles are plasticized with from 1 to 100 parts of plasticizer per part of polymer, and the plasticizer is:

(a) a beta-cyanoethyl ether of a polyhydric aliphatic alcohol, or

10



20

25

where  $\text{R}_3$  and  $\text{R}_4$  are alkyl, cyanoalkyl or phenyl and each  $n$  is a number from 1 to 20.

2. The combination of claim 1 in which the plasticizer is a beta-cyanoethyl ether of a polyhydric alcohol having up to ten carbon atoms and two to four alcohol groups.

3. The combination of claim 1 in which the plasticizer is



in which  $\text{R}_1$  and  $\text{R}_2$  are hydrogen, alkyl containing up to six carbon atoms, or aryl.

4. The combination of claim 1 in which the plasticizer is (b) where  $\text{R}_3$  and  $\text{R}_4$  are alkyl with up to 18 carbons or cyanoethyl and each  $n$  is a number from 1 to 10.

## References Cited

## UNITED STATES PATENTS

|           |         |                  |       |           |
|-----------|---------|------------------|-------|-----------|
| 2,401,607 | 6/1946  | Bruson           | ----- | 260—465.6 |
| 3,079,257 | 2/1963  | Morcher et al.   | ----- | 96—48     |
| 3,158,643 | 11/1964 | Fulmer et al.    | ----- | 260—32.4  |
| 3,219,616 | 11/1965 | Saxon            | ----- | 260—32.4  |
| 3,364,044 | 1/1968  | Grabhofer et al. | ----- | 96—114    |
| 3,364,285 | 1/1968  | Grabhofer et al. | ----- | 96—114    |

## FOREIGN PATENTS

|         |        |                |
|---------|--------|----------------|
| 922,251 | 3/1963 | Great Britain. |
| 926,689 | 5/1963 | Great Britain. |
| 933,391 | 8/1963 | Great Britain. |
| 752,791 | 7/1956 | Great Britain. |

J. TRAVIS BROWN, *Primary Examiner.*

CAROLYN E. DAVIS, *Assistant Examiner.*

U.S. Cl. X.R.

96—48, 67, 87, 114